

Dec. 15, 1925.

1,566,127

W. RUNDQUIST

GLASS LENS AND METHOD OF TREATING THE SAME

Filed Nov. 3, 1924

Fig. 1.



Fig. 2.



Fig. 3.



William Rundquist.

Inventor

By Edson & Symons  
his attorneys

## UNITED STATES PATENT OFFICE.

WILLIAM RUNDQUIST, OF ELGIN, ILLINOIS.

## GLASS LENS AND METHOD OF TREATING THE SAME.

Application filed November 3, 1924. Serial No. 747,591.

*To all whom it may concern:*

Be it known that I, WILLIAM RUNDQUIST, a citizen of the United States of America, residing at Elgin, in the county of Kane and 5 State of Illinois, have invented certain new and useful Improvements in Glass Lenses and Methods of Treating the Same, of which the following is a specification.

My invention relates to improvements in 10 glass lenses or the like, and to methods of treating and preparing the same.

An important object of my invention is to provide a lens so treated that all glare will be eliminated without consequent loss 15 of illumination.

Another object of my invention is the provision of a new and improved method of treating lenses.

Other objects and advantages of my invention will be apparent during the course 20 of the following description.

In the accompanying drawings which form a part of this specification and wherein like characters of reference denote like 25 or corresponding parts throughout the same:

Figure 1 is a front elevation of an automobile headlight provided with my improved lens;

Figure 2 is a section on the line 2—2 of 30 Figure 1; and

Figure 3 is a sectional view of a portion of a lens, illustrating more or less diagrammatically the method of treatment.

In the drawings wherein for the purpose 35 of illustration is shown a preferred embodiment of my invention, the numeral 10 designates an automobile headlight of the usual construction having a bulb 11 arranged therein and provided with a lens 12 arranged in front of said bulb.

Heretofore it has been customary to treat the surface of lenses by sand blasting, for the purpose of cutting down the glare, but this treatment is such that a frosting or 45 coating is formed on the surface of the lens, which prevents the light from getting through, or in other words, "bottles" it. This sandblasting is done by projecting the sand upon the lens at an angle perpendicular to the surface of the lens, as illustrated by the dotted arrows A in Figure 3 of the drawing.

Because of this angle, it is impossible to exert any great amount of

pressure on the sand because of breaking the lens. 55

I have discovered, however, that if coarse particles of silica of a uniform size are projected against the inner surface of the lens under great pressure and at an angle substantially less than 90 degrees with respect 60 to the surface of the lens to be treated as illustrated by the arrows B in Figure 3, the frosting does not appear on the finished lens. By directing the silica blast at an angle less than a right angle, great force may 65 be employed, without breaking the lens. The large uniform particles of silica projected in a slanting stream, groove the surface of the lens and affect the very texture of the glass by crushing the fine cells or 70 globules within the lens. Flakes are cut out slantingly which force the light to pass sideways through the lens.

When the coarse particles of silica strike the glass with great force, the interior, as 75 well as the surface, is affected, substantially regular crystals being formed within the glass by reason of the uniformity in size of the silica particles. The sides of these crystals, within the glass, are snowy white, 80 and the light passing therethrough is changed from a clear to a milky white. These crystals, together with the flakes cut out of the surface, sift the white light and 85 diffuse it. The light is not bottled up, but is all allowed to go through the lens. The coating formed by a perpendicular stream of fine sand, or sand containing some fine particles is not formed by my process of 90 treating the glass because of the uniformity of the size of the silica particles, the great amount of pressure, and the direction in which the silica is projected against the surface of the glass.

Heretofore it has been usual to use what is known by the trade as pressed glass for nonglare lenses. With my method of treatment, however, it is possible to use drawn glass without any danger of 95 glare. By treating the inside surface of the lens, the cause of glare is attacked at its source, and the crystals throw beams of 100 nonglaring light through the remainder of the clear glass.

Lenses treated with my improved method, cut out all glare with no consequent loss 105

of illumination and therefore portions of clear, untreated glass are rendered unnecessary, thereby dispensing with a dangerous feature of many types of lenses which so bottle up the light that it is necessary to let the light out without diffusing it, in portions of the glass.

While I have shown and described my invention as applicable to automobile lenses, 10 it is to be understood that I do not limit myself to this use, as I have discovered it useful in window lighting and other arts.

Having described my invention what I 15 claim and desire to protect by Letters Patent is:

1. The method of treating glass lenses which consists in directing a blast of silica at an angle to the surface of the lens.
2. The method of treating lenses which 20 consists in projecting a stream of uniform particles of silica in a slanting direction upon the surface of the lens.
3. The method of treating lenses which 25 consists in projecting a slanting stream of coarse particles of silica with a great amount of force, upon the surface of the

lens, to form substantially uniform crystallized surfaces within the texture of the lens by breaking up the globules of the glass.

4. A lens having its surface treated with 30 silica blasting whereby the globules of the glass are broken up into regular crystals, each of said crystals being adapted to throw a separate beam of light, thereby doing away with all glare.

5. A lens having its inner surface treated to form crystallized surfaces radiating towards the interior of the lens, said crystallized surfaces being of a color to change 35 the light to a milky color.

6. A lens having its inner surface treated to form slanting grooves on the surface and crystallized surfaces radiating towards the interior of the lens, whereby light going 40 through the lens will be broken up and diffused.

7. A lens having one of its surfaces smooth and the other surface treated to form crystallized surfaces radiating towards 45 the interior of the lens.

In testimony whereof I affix my signature.

WILLIAM RUNDQUIST.